

1,302,512.

A. L. CLAPP.

GUN WAD FELT AND PROCESS OF MAKING,  
APPLICATION FILED MAY 27, 1915. RENEWED APR. 1, 1916.

Patented May 6, 1919.

Fig. 1.



Fig. 2.



Fig. 3.



Fig. 4.



Inventor:

Albert L. Clapp,  
by *Geo. St. Marie*  
Attorney.

# UNITED STATES PATENT OFFICE.

ALBERT L. CLAPP, OF BRAINTREE, MASSACHUSETTS, ASSIGNOR TO THE METALITE COMPANY, OF AMESBURY, MASSACHUSETTS, A CORPORATION OF DELAWARE.

## GUN-WAD FELT AND PROCESS OF MAKING.

1,302,512.

Specification of Letters Patent.

Patented May 6, 1919.

Application filed May 27, 1915, Serial No. 30,764. Renewed April 1, 1916. Serial No. 88,396.

To all whom it may concern:

Be it known that I, ALBERT L. CLAPP, a citizen of the United States, and resident of Braintree, in the county of Norfolk and State of Massachusetts, have invented an Improvement in Gun-Wad Felt and Processes of Making, of which the following description, in connection with the accompanying drawings, is a specification, like letters on the drawings representing like parts.

My present invention is an improved article of manufacture, intended particularly for use in waddings for guns, cartridges, or the like, and consists in such an improved article and in the novel process of making the same.

In the accompanying drawing, Figures 1 and 2 represent the pressed sheet and Figs. 3 and 4 the gunwads.

In the manufacture of wadding material for use in cartridges, and firearms generally, the material, as heretofore made, is expensive, consisting in a mixture of animal hair, glue, and flour, being made on a fulling machine, such as is ordinarily employed in felt-  
ing. It will be readily appreciated that in this particular art, *i. e.*, wadding for firearms, a highly resilient material is necessary, which will pack down firmly between the charge of powder and the bullet, shot, or the like, and yet which will not change its condition nor disintegrate during long periods of time. It has been customary to make such wadding material on a fulling machine, as above explained, and then to cut the wads from the rough sheets thus made. A great objection to the old style material is that the mixture of hair, glue, and flour necessary, results in hardening the hair in a short time, rendering it unelastic and not suitable for use. As a great deal of this wadding is made up in cartridges and must be held in stock for long periods before shipment or use, the inefficiency of such wadding through the change due to hardening and brittleness of the hair renders it unsuitable and unsatisfactory in many cases.

I have discovered that I can produce an article of manufacture which is especially suitable for gun-wadding at a fraction of the expense heretofore involved in old-style processes and materials, and which is also lighter and of higher resiliency. I utilize a mixture of animal hair and wood pulp,

treating both the wood pulp and hair in a particular manner, mixing them in an ordinary beater, but in a particular way, and forming a sheet of felt-like material in a mold where it is screened, dried, and subsequently pressed. In carrying out this invention, I am enabled to use from 20 to 40% of wood pulp, which is very inexpensive, grinding such wood pulp in an ordinary beater and treating it with a small percentage, approximately 5%, of caustic soda, which renders the wood pulp soft and also makes it fluffy. I then treat the remaining proportion of animal hair in a similar beater, but with the beating knives so set as not to cut the hair material, allowing it to slip through the cutting knives and thus preserve the fiber. With the hair thus in the beater I also add a small percentage of caustic soda, soap, or an equivalent, which still further preserves the fiber or the hair from injury by facilitating its slipping by the beater knives, and straightening out as the hair is dumped into a mold. With the wood pulp and hair thus separately treated, I then mix the desired portions in a common beater, preferably pouring the wood pulp in the beater in which the hair has been treated so as to insure that the beater knives will not damage the fiber of the hair. During mixing, I prefer to add a small percentage of animal sizing, for example 10% of casein, which constitutes a binder and gives firmness and tenacity to the entire product. This product is then dumped into a mold having a suitable screen to drain out the water, and preferably a plunger or the like is applied to the mass in the mold to further squeeze out the water; after which the sheet material is dried, and preferably again repressed. As thus made, my improved material is extremely light and will maintain its resiliency through long periods of time, especially when made up into gun wadding in cartridges. Furthermore, I am enabled to use any sort, or kind, or grade, or length of hair, waste hair, and the like, in my process, whereas in the prior manufacture of gun wadding it was essential to use a high grade and expensive goat hair. With the sheets of felt thus made and repressed the desired size and diameter of wadding is cut therefrom in the usual manner.

I have explained my invention, compris-

ing both the novel form of article and the process of making the same, as for the manufacture of wadding material for cartridges, guns, etc., but it will be understood that this 5 is only one of the many uses for which my inventions may be utilized.

The important feature consists in the combination of a resilient felt-like material of wood pulp and hair mixed, prepared and 10 treated in a novel manner. The resulting product is useful for all purposes where any kind of resilient felt-like material is desired, such as in upholstery, electrical insulation uses, sound and vibration deadening, pack- 15 ings of various kinds, insoles and shoe fillers, and in numerous other applications wherein felt-like sheets, blocks or material can be used.

Having described my invention, what I 20 claim as new and desire to secure by Letters Patent is:

1. As an improved article of manufacture, a gun-wad felt consisting in the mixture of a quantity of hair treated with a small percentage of caustic soda, a proportion of wood pulp from 20% to 40% in quantity of the prepared hair, separately treated with a small percentage of caustic soda, and both quantities mixed throughout with binding 30 and adhesive agent, and molded into sheets.

2. The process of making gun-wad felt, which consists in treating a quantity of animal hair in a beating machine with a small percentage of caustic soda, and adding 35 thereto 20% to 40% of wood pulp, mixing said hair so treated with said wood pulp, treating both said quantities during further mixing with a small percentage of animal sizing, pouring the combined mixture into 40 a mold, draining the water therefrom and drying the molded product.

3. The process of making gun-wad felt, which consists in treating a quantity of animal hair in a beating machine with approximately 45 5% of caustic soda but so as to retain substantially the original length of the hair, and then beating a quantity of wood pulp, simultaneously treating it with approximately 5% of caustic soda, then mixing both 50 hair thus treated and the wood pulp thus treated in the proportion of 60% to 80% of hair to 20% to 40% of wood pulp, and treating the mass thus mixed with approximately 10% of casein, pouring the combined 55 mixture into a mold, draining the water therefrom and drying the molded product, and then subjecting the same to a pressing

action to solidify and form it into sheets of desired thickness.

4. As an article of manufacture, a felt-like material consisting in the mixture of animal hair and fibrous pulp treated with an alkali and thoroughly intermixed in the presence of water and dried to form a light, 60 resilient mass.

5. As an article of manufacture, a resilient felt-like material consisting of an intimate mixture of alkali-treated animal hair and fibrous pulp with a binder.

6. That process of making felt-like material, which is characterized by treating fibrous cellulose with water and a caustic alkali; treating the mixture of fibrous cellulose and caustic alkali in water thus obtained to reduce the fibrous cellulose to a finely 75 divided state; treating animal hair in water with a caustic alkali; thoroughly intermixing the aqueous mixture of alkali and animal hair thus obtained with the aqueous mixture of alkali and finely divided fibrous 80 cellulose; thoroughly mixing with the mixture thus obtained a suitable sizing material; forming the stock thus obtained into sheets; and drying and pressing said sheets.

7. That process of making felt-like material which is characterized by treating fibrous cellulose and animal hair with a solution of alkali, reducing the fibrous cellulose to a relatively finely divided state and thoroughly intermixing said fibrous cellulose 90 with the animal hair; adding to the mixture thus obtained and thoroughly intermixing therewith at some time during the process, a suitable sizing material; and forming the stock thus obtained into sheets.

8. That process of making felt-like material, which is characterized by treating fibrous stock and animal hair with a solution of alkali, reducing the fibrous stock to a relatively finely divided state and thoroughly 100 intermixing said fibrous stock with the animal hair; adding to the mixture thus obtained and thoroughly intermixing therewith at some time during the process, a suitable sizing material; and forming the stock 105 thus obtained into sheets.

In testimony whereof, I have signed my name to this specification, in the presence of two subscribing witnesses.

ALBERT L. CLAPP.

Witnesses:

GEORGE E. SAMPSON,  
HENRIETTA NEAL.